

2,861,065

## ARYLGUANIDINE ARENEDIAZOSULFONATES

Clifford E. Herrick, Jr., Chenango Forks, N. Y., assignor to General Aniline & Film Corporation, New York, N. Y., a corporation of Delaware

No Drawing. Application December 31, 1956  
Serial No. 631,424

6 Claims. (Cl. 260—141)

The present invention relates to arylguanidine arenediazosulfonates which are photosensitive, solvent-soluble compounds having particular utility in the manufacture of light-sensitive diazotype materials and lithographic plates.

It has become increasingly apparent in recent years that high molecular weight, photosensitive compounds which are soluble in organic solvents, such as alcohols, esters, ketones, methyl Cellosolve, dimethylformamide, chloroform and the like, have important applications in the diazotype and lithographic fields. Representative of such compounds on which considerable work has already been done are the diazoxydes, diazoimides, 3-diazoindoles, 3-diazoindazoles and nitrones. Each of these fills an important segment of the involved fields, but considerable research is under way to find new compounds serving to bridge the hiatus in said fields which cannot be served adequately by the presently known compounds.

It has now been discovered that arylguanidine arenediazosulfonates, which are salts of high molecular weight, are photosensitive, solvent-soluble substances having such characteristics. These compounds, because of their attributes, are particularly suitable for use in lithography, i. e., in the manufacture of paper and metal lithographic plates.

Arylguanidine arenediazosulfonates, their preparation and their use in diazotype and lithography constitute the purposes and objects of the present invention.

The new general class of photosensitive, solvent-soluble substances contemplated herein is typified by the following general formula:



wherein Ar is an aromatic radical such as phenyl or substituted phenyl, i. e., alkylphenyl such as methylphenyl, ethylphenyl and the like; alkoxyphenyl such as methoxyphenyl, ethoxyphenyl, dimethoxyphenyl, diethoxyphenyl, dipropoxyphenyl, dibutoxyphenyl and the like; halophenyl such as chlorophenyl, bromophenyl and the like; alkylaminophenyl such as methylaminophenyl, ethylaminophenyl, N,N-dimethylaminophenyl, N,N-diethylaminophenyl, N-ethyl-N-propylaminophenyl, N-ethyl-N-butylaminophenyl, N-ethyl-N-β-hydroxyethylaminophenyl, N-ethyl-N-benzylaminophenyl and the like; cycloalkylaminophenyl such as cyclohexylaminophenyl and the like; arylaminophenyl such as phenylaminophenyl, N-phenyl-N-naphthylaminophenyl and the like; acylaminophenyl such as acetylaminophenyl, phenylthioacetylaminophenyl, benzoylaminophenyl, phenylacetylaminophenyl and the like; and phenoxyphenyl; phenylthiophenyl; diphenyleneoxide; naphthyl; diphenylenesulfide; benzylphenyl, phenethylphenyl and such aromatic radi-

cals starting with said phenoxyphenyl as bear the same substituents as those listed for the phenyl radicals; R being hydrogen or aryl such as phenyl; alkylphenyl such as methylphenyl, dimethylphenyl and the like; naphthyl such as 1- or 2-naphthyl and the like, at least two R's being aryl and at least one R being hydrogen.

The new salts are made by preparing in a known manner the required alkali metal arenediazosulfonate and reacting the same in an aqueous medium with the selected arylguanidine acetate with gentle heating if desired. The arylguanidine arenediazosulfonates separate from the aqueous solution, sometimes as solids, sometimes as oils which later crystallize. The photosensitive solids which have a color ranging from yellow to orange, red or brown are insoluble in water but soluble in such solvents as isopropyl alcohol, acetone and chloroform. They may be, accordingly, coated on a suitable base from such solvents to prepare diazotype and lithographic materials.

- 20 Examples of the arenediazosulfonates which are suitable for the preparation of the photosensitive compounds are the alkali metal salts such as sodium p-ethoxybenzenediazosulfonate; sodium 3-chloro-4,6-dimethoxybenzenediazosulfonate; sodium p-acetamidobenzenediazosulfonate; sodium N-benzyl-N-ethyl-p-aminobenzenediazosulfonate; sodium 2,5-diethoxy-4-methylbenzenediazosulfonate; sodium 2,5-dimethoxybenzenediazosulfonate; sodium 4-bromo- or chloro-2,5-diethoxybenzenediazosulfonate; sodium 5-chloro-2,4-diethoxybenzenediazosulfonate; sodium 2-chloro-4,5-dimethoxybenzenediazosulfonate; sodium 4-diethylamino-6-ethoxybenzenediazosulfonate; sodium 4-diethylamino-2,6-diethoxybenzenediazosulfonate; sodium 4-dimethylamino-6-methoxybenzenediazosulfonate; sodium N-ethyl-N-propyl-4-amino-6-ethoxybenzenediazosulfonate; sodium N-ethyl-N-β-hydroxyethyl-4-amino-6-ethoxybenzenediazosulfonate; sodium 4-ethyl-amino-3-methylbenzenediazosulfonate; sodium 4-diethylaminobenzenediazosulfonate; sodium N-ethyl-N-benzyl-4-aminobenzenediazosulfonate; sodium N-ethyl-N-β-hydroxyethyl-4-aminobenzenediazosulfonate; sodium 4-dimethylaminobenzenediazosulfonate; sodium 4-benzylamino-2-methoxy-5-methylbenzenediazosulfonate; sodium 4-benzoylamino-2-methoxy-5-methylbenzenediazosulfonate; sodium 4-benzoylamino-2-chloro-5-methoxybenzenediazosulfonate; sodium 4-(4'-methoxyphenylamino)benzenediazosulfonate; sodium 4-phenylthioacetyl-amino-2,5-diethoxybenzenediazosulfonate; sodium 4-cyclohexylaminobenzenediazosulfonate; sodium 2,4,5-triethoxybenzenediazosulfonate; sodium 4-acetylamino-2,5-dibutoxybenzenediazosulfonate; sodium 4-phenylacetyl-amino-2,5-diethoxybenzenediazosulfonate; sodium 4-ethylmercapto-2,5-diethoxybenzenediazosulfonate; sodium 4-ethylmercapto-2,5-diethoxybenzenediazosulfonate; sodium 4-morpholinobenzenediazosulfonate; sodium 4-β-naphthylaminobenzenediazosulfonate; disodium 3,3'-dimethoxy-4,4'-biphenyltetrazodisulfonate; disodium 4,4'-biphenyltetrazodisulfonate; sodium 4-tolyl-2,5-diethoxybenzenediazosulfonate; sodium 4'-acetylamino-2,5-diethoxy-4-biphenyl diazosulfonate; sodium 4'-2,5-triethoxy-4-biphenyl diazosulfonate; sodium 4'-ethoxy-2,5-dibutoxy-4-biphenyl diazosulfonate; sodium 1-naphthalenediazosulfonate; sodium 2-naphthalenediazosulfonate; the tetrazodisulfonate from 4,4'-diaminodiphenyleneoxide; the tetrazodisulfonate from 4,4'-diaminodiphenylenesulfide; the sodium diazosulfonate from 4'-amino-m-terphenyl; disodium 3,3'-methylenebis(4-ethoxybenzenediazosulfonate); disodium 3,3'-ethylenebis(4-ethoxybenzenediazosulfonate); the sodium tetrazodisulfonate from p,p'-ethylenediaminoaniline and the like.

70 The arylguanidines which are reacted with any of the aforesaid diazosulfonates to produce the photosensitive

3

compounds hereof are those of the following general formula:



wherein R is hydrogen or an aromatic radical of the benzene or naphthalene series such as phenyl, alkylphenyl, i. e., tolyl, xylol or the like; acylaminophenyl such as lauroylaminophenyl and the like; alkylsulfamoylphenyl such as dodecylsulfamoylphenyl and the like; naphthyl such as 1-naphthyl, 2-naphthyl and the like, it being understood that at least two R's are such aromatic radicals and at least one R is hydrogen.



Illustrative of such arylguanidines are:

1,3-di-o-tolylguanidine  
1,3-dixylylguanidine  
1,2,3-triphenylguanidine  
1,1,2,3-tetraphenylguanidine  
1,2-diphenyl-3-o-tolylguanidine  
1-(p-lauroylaminophenyl)-3-phenylguanidine  
1-(p-dodecylsulfamoylphenyl)-3-phenylguanidine  
1,3-di-1-naphthylguanidine  
1,3-di-2-naphthylguanidine  
1,3-diphenyl-2(1-naphthyl)guanidine, and the like.



The invention is further illustrated by the following examples, but it is to be understood that the invention is not restricted thereto.

#### Example I

175 gms. of sodium p-ethoxybenzenediazosulfonate was dissolved by gentle heating in a mixture of 1750 mls. of water and 70 mls. of acetic acid. To the above solution was added a solution of 175 gms. of 1,3-di-o-tolylguanidine in 700 mls. of water and 620 mls. of acetic acid.

A heavy yellow precipitate formed upon slow addition with stirring at 35-40° C. The slurry was cooled to 18-20° C. and filtered. The cake was then slurried twice with water, re-filtered and dried in vacuo over sodium hydroxide. The yield was 90 percent. The crystals melted at 147-149° C.

The probable structure of the product is:



#### Example II

Thirty grams of sodium 3-chloro-4,6-dimethoxybenzenediazosulfonate was dissolved in one liter of water plus 20 mls. of glacial acetic acid. A little methanol was added. The material did not entirely dissolve and was filtered. To the filtrate was added a solution of 24 grams of 1,3-di-o-tolyl guanidine in 150 mls. of 50% acetic acid.



4

acid. A red oil appeared. This oil was washed with water and left for two days. Some yellow crystals were observed on the third day. On the fourth day crystallization occurred. The crystals were washed with water, filtered, and dried in vacuo. The crystals melted at 162-164° C. The yield was 72%.

The probable structure is:



#### Example III

15 1,3-di-o-tolylguanidine 3,3'-dimethoxy-4,4'-biphenyltetrazodisulfonate was prepared in the same manner as in Example I. The reddish yellow crystals melted at 153-155° C. with decomposition and probably possessed the following structure:



#### Example IV

25 1,3-di-o-tolylguanidine 4,4'-biphenyltetrazodisulfonate was prepared from sodium biphenyltetrazodisulfonate in the same manner as in Example I. The sodium biphenyltetrazodisulfonate was made by tetrazotizing benzidine and treating the solution with solutions of sodium bicarbonate and sodium sulfite.

The structure of the product is probably:



#### Example V

40 A solution of 17.5 grams of sodium p-acetamidobenzenediazosulfonate in 50 mls. of warm water was treated with a warm solution of 33.5 grams of 1,3-di-o-tolylguanidine in 100 mls. of acetic acid, 50% by volume. An oil separated which solidified to orange crystals when refrigerated. These were collected, washed, and dried in vacuo. The product weighed 28.0 grams, an 84% yield, melted with decomposition at 176-180° C. and probably had the structure:



#### Example VI

55 2,2'-methylenebis(4-nitrophenol) (Chattaway and Goepp, J. Chem. Soc. 1933, 699) was converted by means of ethyl sulfate and alkali into 2,2'-methylenebis(4-nitrophenol), which was reduced catalytically over palladium on carbon to 3,3'-methylenebis(p-phenetidine). The hydrochloride of this base was diazotized and converted to sodium 3,3'-methylenebis(4-ethoxybenzenediazosulfonate) in the usual way.

60 A filtered solution of 18.5 grams of sodium 3,3'-methylenebis(4-ethoxybenzenediazosulfonate) in about 500 mls. of water was treated with 38 grams of 1,3-di-o-tolylguanidine in 100 mls. of water and 100 mls. of acetic acid. The product separated as a yellowish-brown mass, weight 12 grams, decomposition point 135° C. after softening at 80° C. The structure is probably:



## Example VII

A filtered solution of 36.0 grams of N-benzyl-N-ethyl-p-aminobenzenediazonium chloride zinc chloride double salt was treated with a solution of 25.2 grams of sodium sulfite in 100 mls. of water. The yellowish-orange crystals of sodium N-benzyl-N-ethyl-p-aminobenzenediazosulfonate were collected, dissolved in 100 mls. of water and 5 mls. of acetic acid, treated with a warm solution of 35.8 grams of 1,3-di-o-tolylguanidine in about 100 mls.



of acetic acid, 50% by volume. The yellow crystalline product, after being filtered, washed and dried in vacuo, weighed 18.3 grams, a 33% yield, melted at 175-8° C. and was very sensitive to light. The probable formula is:



Modifications of the invention will occur to persons skilled in the art. Thus, it is to be particularly pointed out that any of the diazosulfonates listed herein may be reacted by the procedures of the samples with any of the arylguanidines to yield the photosensitive products. I, therefore, do not intend to be limited in the patent granted except as necessitated by the prior art and the appended claims.

I claim:

1. Photosensitive compounds soluble in organic solvents having the following formula:



wherein Ar is selected from the class consisting of aromatic radicals of the benzene and naphthalene series and heterocyclic radicals of the diphenyleneoxide and diphenylenesulfide series, R is selected from the class consisting of hydrogen and an aromatic radical of the benzene and naphthalene series, at least two R's being such an aromatic radical and at least one R being hydrogen.

2. A photosensitive compound soluble in organic solvents having the following formula:



3. A photosensitive compound soluble in organic solvents having the following formula:



4. A photosensitive compound soluble in organic solvents having the following formula:



5. The process of producing photosensitive compounds soluble in organic solvents and having the following structural formula:



wherein Ar is selected from the class consisting of aromatic radicals of the benzene and naphthalene series and heterocyclic radicals of the diphenyleneoxide and diphenylenesulfide series and R is selected from the class consisting of hydrogen and an aromatic radical of the benzene and naphthalene series, at least two R's being such an aromatic radical and at least one R being hydrogen, which comprises reacting an alkali metal arenediazosulfonate in an aqueous medium with the acetate of an arylguanidine of the following formula:



in which R is selected from the class consisting of hydrogen and an aromatic radical of the benzene and naphthalene series, at least two R's being such an aromatic radical and at least one R being hydrogen.

6. The process as defined in claim 5, wherein the arenediazosulfonate is sodium p-ethoxybenzenediazosulfonate and the arylguanidine acetate is the acetate of 1,3-di-o-tolylguanidine.

No references cited.